

## United States Patent Office

2,880,055

Patented Mar. 31, 1959

1

2,880,055

## METHOD OF REDUCING THE ALKALI SOLUBILITY OF WOOL BY TREATMENT WITH ACROLEIN

George Thomson, Milton, Carter G. Cook, Norwood, and Phyllis M. Pepin, Hyde Park, Mass., assignors to Fabric Research Laboratories, Inc., Boston, Mass., a corporation of Massachusetts

No Drawing. Application July 15, 1953  
Serial No. 368,226

4 Claims. (Cl. 8—133)

The present invention relates to the treatment of wool and other keratinous materials, and consists in a process for counteracting the effects of chemical degradation of such materials.

Chemical degradation of wool is caused by many of the treatments to which it is subjected during its processing, particularly treatments under acidic, oxidizing, or reducing conditions, and results in an impairment of the physical or mechanical properties of the wool. During carbonization, for instance, wool is treated with sulfuric acid and baked to remove foreign vegetable matter, and acid conditions are also frequently encountered during dyeing, and during decolorizing processes such as the electrolytic stripping process disclosed in U.S. Patent No. 2,549,099. Such treatments under acidic conditions result in acid damage to the wool, believed to be caused by the hydrolysis, and consequent breaking, of peptide links present in the wool molecule.

Decolorizing and bleaching treatments subject the wool to oxidizing or reducing conditions that also result in degradation of the wool, believed to be caused by the breakage of cystine links in the molecular structure.

The degree of degradation is commonly measured by the alkali solubility, which is increased by degradation. The alkali solubility values used in this disclosure were obtained by immersing a 1 gram sample of the wool in 100 cc. of a 0.1 N aqueous sodium hydroxide solution at a temperature of 65° C. for one hour, then filtering out the wool, rinsing it thoroughly with water and drying.<sup>1</sup> The loss of weight expressed as a percentage of the original weight is the alkali solubility value, and is a generally accepted index to the degree of degradation.

The effect of various degradation-causing treatments of samples of virgin Australian wool and of samples of a commercial blue-dyed yarn are shown in Table I.

TABLE I

| Sample                                                                                                                               | Alkali Solubility, Percent |
|--------------------------------------------------------------------------------------------------------------------------------------|----------------------------|
| 1. New Virgin Australian Raw Wool                                                                                                    | 13.1                       |
| 2. Sample 1 after boiling for 1 hr. in 0.1 N HCl                                                                                     | 45.2                       |
| 3. Sample 1 after bleach in commercial 6% H <sub>2</sub> O <sub>2</sub> for 1/4 hr. at 65° C.                                        | 39.6                       |
| 4. Sample 3 after boiling for 1 hr. in 0.1 N HCl                                                                                     | 67.0                       |
| 5. A commercial blue-dyed wool yarn                                                                                                  | 11.8                       |
| 6. Sample 5 after electrolytic strip in 5% sulfuric acid solution (a reducing treatment), as described in U. S. Patent No. 2,549,099 | 69.2                       |

The present invention provides a process for treating wool, and other keratinous materials, to enhance its resistance to degradation or to recondition wool that has been damaged, and is effective in counteracting the

2

damaging effects of treatments under acidic, oxidizing, or reducing conditions.

The process of this invention consists essentially in treating the material in an aqueous solution of acrolein, an unsaturated aldehyde having the structure



10 The treatment may be carried out effectively in solutions containing as little as 0.3 percent by weight of acrolein, but higher concentrations in the range of about 3 to about 6 percent by weight of acrolein are preferred, as they produce better results at a faster rate. Higher concentrations of acrolein are also entirely satisfactory, but unnecessary, for no significant additional improvements in the treatment have been found to result from increasing the acrolein concentration above about 6 percent. The treating solution is preferably neutral or slightly acid, and is accordingly adjusted to have a pH in the range of about 2-7.

15 The treatment may be carried out at ordinary temperatures between the freezing point and boiling point 25 of the solution, or at even such higher temperatures as are not destructive to the keratinous materials if pressure systems are to be used. When wool is treated in accordance with this invention to repair damage previously caused by overbleaching, a treatment at a 30 temperature above 65° C. is more effective than lower temperatures to stabilize the wool against subsequent acid damage, and such higher temperatures are accordingly preferred for this type of treatment.

20 The time required for the treatment is interrelated 35 with the temperature and concentration, but under the preferred conditions the treatment is ordinarily complete in less than 2 hours, and about 20 minutes is generally adequate. It will be understood, however, in accordance with well known principles of chemical kinetics, that longer or shorter periods of time may be preferred under some conditions depending in part on the acrolein concentration, temperature and degree of damage-counteraction desired.

25 Where whiteness of the wool is desired, it is preferable to add to the treating solution, in addition to the acrolein, a small amount of methacrolein. Acrolein alone in solution has some tendency to cause yellowing. In a solution containing 3 percent by weight of acrolein, the addition of about 2 percent by weight of methacrolein reduces the tendency toward yellowing, and also prevents darkening of the wool at elevated temperatures. In this connection it has been found that the addition of formaldehyde to the acrolein solution is also effective to diminish the tendency of the wool 50 to become yellow.

30 In carrying out the process the keratinous material is simply immersed in the acrolein solution, then removed and dried. The material may be rinsed prior to final drying, but this is not necessary, and when treating wool 35 damaged by overbleaching, it is advantageous to leave the wool unrinsed and to dry at elevated temperatures such as do not cause damage to the wool, for instance, 60-120° C. or even higher for short duration.

35 Representative examples of the process of this invention, presented as illustrative of the best manner now known of carrying it out, and the results thereof are 40 reported in Table II. In each example, a sample of wool was immersed in the acrolein solution, then removed, rinsed (except where noted), and dried under the 45 conditions given in the table. Under the heading "Bath Ratio" is given the parts by weight of solution per part of dry wool. The pH in each example was adjusted by

<sup>1</sup> See Von Bergen and Mauersberger, American Wool Handbook, 2nd ed. (1948) (Textile Book Publishers, Inc., N.Y.), p. 951.

adding acetic acid to the solution to lower the pH, or soda ash to raise the pH.

After each treatment, the alkali solubility of the sample was determined both before and after the sample was boiled for one hour in an aqueous 0.1 N hydrochloric acid solution, and the results tabulated indicate both the degree by which the treatment improved the alkali solubility and the degree by which it stabilized the wool against subsequent acid damage. For comparison, the alkali solubility figures are also given for the samples before treatment, under the heading "Control."

pH of 6 at a temperature maintained between 40-45° C. for 90 minutes. The wool was then removed, rinsed and dried at 100° C. The alkali solubility was determined to be 14.3%.

In the following example a solution of acrolein and formaldehyde was used to pretreat a dyed wool prior to electrolytic stripping, to minimize subsequent damage from the combination of acidic and reducing conditions during stripping.

*Example 19*

The blue dyed wool yarn reported in Table I (item 5)

TABLE II

|                 | Type of Wool                                   | Conditions of Treatment |            |    |            |            | Drying | Alkali Solubility |                 |
|-----------------|------------------------------------------------|-------------------------|------------|----|------------|------------|--------|-------------------|-----------------|
|                 |                                                | Acrolein Conc., Percent | Bath Ratio | pH | Temp., °C. | Time, Min. |        | Before Acid Boil  | After Acid Boil |
| Control I.....  | Virgin Australian Wool, Washed and De-greased. |                         |            |    |            |            |        | 13.1              | 45.2            |
| Example:        |                                                |                         |            |    |            |            |        |                   |                 |
| 1.....          | do.....                                        | 3                       | 30         | 3  | 20         | 20         | 20     | 8.6               | 19.6            |
| 2.....          | do.....                                        | 0.3                     | 100        | 3  | 20         | 20         | 100    | 11.7              | 35.2            |
| 3.....          | do.....                                        | 5                       | 20         | 3  | 20         | 20         | 100    | 8.3               | 19.4            |
| 4.....          | do.....                                        | 10                      | 10         | 3  | 20         | 20         | 100    | 8.3               | 18.9            |
| 5.....          | do.....                                        | 3                       | 30         | 3  | 65         | 20         | 100    | 8.5               | 16.4            |
| 6.....          | do.....                                        | 3                       | 30         | 3  | 85         | 20         | 100    | 8.8               | 13.7            |
| 7.....          | do.....                                        | 3                       | 30         | 3  | 100        | 20         | 100    | 7.6               | 12.8            |
| 8.....          | do.....                                        | 3                       | 30         | 3  | 20         | 10         | 100    | 9.0               | 20.3            |
| 9.....          | do.....                                        | 3                       | 30         | 3  | 20         | 60         | 100    | 7.3               | 16.0            |
| 10.....         | do.....                                        | 3                       | 30         | 3  | 100        | 10         | 100    | 6.3               | 13.8            |
| 11.....         | do.....                                        | 3                       | 30         | 3  | 100        | 60         | 100    | 6.5               | 12.0            |
| Control II..... | Commercial Over-bleached White Yarn.           |                         |            |    |            |            |        | 47.1              | 74.5            |
| Example:        |                                                |                         |            |    |            |            |        |                   |                 |
| 12.....         | do.....                                        | 3                       | 30         | 3  | 20         | 20         | 20     | 22.6              | 68.2            |
| 13.....         | do.....                                        | 3                       | 30         | 3  | 20         | 20         | 100    | 24.8              | 42.5            |
| 14.....         | do.....                                        | 3                       | 30         | 3  | 100        | 20         | 100    | 14.3              | 29.2            |
| 15.....         | do.....                                        | 3                       | 30         | 7  | 100        | 20         | 100    | 13.7              | 26.6            |
| 16.....         | do.....                                        | 3                       | 30         | 7  | 100        | 20         | 100    | 12.2              | 23.6            |

<sup>1</sup> Dried without rinsing the wool after its removal from treating bath.

The foregoing examples demonstrate the wide range of conditions under which the process of this invention may be effectively practiced. It will be seen from Examples 12-16 that in reconditioning an overbleached yarn, best results are obtained when the wool is treated at a high temperature, and dried at a high temperature, and that a pH of 7 is apparently better than a lower one. Under these conditions a wool having the alkali-solubility characteristics of an undamaged virgin wool may be obtained.

*Example 17*

The peroxide bleached wool described in Table I (item 3) was immersed for 20 minutes in 30 times its weight of a 3% (by weight) acrolein solution (aqueous) having a pH of 3 to 20° C., then removed, rinsed and dried at 100° C. The alkali solubility of this sample was determined both before and after a 1 hour boil in a 0.1 N HCl solution.

Alkali solubility, percent

Before acid boil ..... 19.5  
After acid boil ..... 44.6

These values, it will be seen, compare favorably with the corresponding values obtained on the unbleached control, 13.1 and 45.2 respectively.

*Example 18*

A dyed carpet wool, having an alkali solubility of 9.9%, was electrolytically stripped in a chromium sulfate solution containing 3% sulfuric acid at a temperature of 85° C., as described in Patent No. 2,549,099. The stripping raised the alkali solubility to 37.9%. The wool was then immersed in a 6% acrolein solution having a

45 was immersed for 20 minutes in 30 times its weight of an aqueous solution having a pH of 6 and containing 3% acrolein (by weight) and 2% formaldehyde (by weight), at a temperature of 25° C., then removed, rinsed and dried at 100° C. The alkali solubility was found to be 8.0%. The treated yarn was then electrolytically stripped in a 5% sulfuric acid solution as described in Patent No. 50 2,549,099. After stripping, the alkali solubility was found to be 23.4%. From Table I it will be seen that without the acrolein treatment the yarn, after the electrolytic strip, had an alkali solubility of 69.2%. The presence of formaldehyde in the pretreating solution substantially diminished yellowing of the yarn.

55 In the following example, samples of virgin Australian wool tops treated with acrolein in accordance with this invention and subsequently electrolytically stripped are compared with respect to their elongation and tensile 60 strength characteristics, with samples of the same wool electrolytically stripped without having been treated with acrolein.

*Example 20*

65 The acrolein treatment consisted in immersing the wool in 30 times its weight of an aqueous 3% (by weight) acrolein solution having a pH of 3, for 20 minutes at room temperature, then drying at 100° C.

The electrolytic stripping process was that described 70 in Pat. No. 2,549,099 and was carried out in an aqueous solution containing 3% (by weight) of sulfuric acid and 2% (by weight) of basic chromium sulfate.

The following results were obtained, using an Instron tensile tester, manufactured by Instron Engineering Co., Quincy, Massachusetts.

|                                                                     | Yield load intensity at 5% elongation, grams/denier | Breaking strength, grams/denier | Elongation at rupture, percent |
|---------------------------------------------------------------------|-----------------------------------------------------|---------------------------------|--------------------------------|
| Control.....                                                        | .89                                                 | 1.48                            | 34.9                           |
| Sample after acrolein treatment.....                                | .83                                                 | 1.29                            | 32.9                           |
| Sample after electrolytic strip.....                                | .81                                                 | 1.20                            | 34.3                           |
| Sample after acrolein treatment followed by electrolytic strip..... | .93                                                 | 1.30                            | 31.6                           |

From these results it will be seen that significant improvements in the wool after an electrolytic strip may be attributed to the acrolein treatment of this invention, particularly with regard to the yield point and the breaking strength.

From the foregoing disclosure, it is apparent that the process of this invention is effective to lessen the degradation encountered when wool is treated under acidic, oxidizing or reducing conditions, and also to counteract degradation previously caused by treatments under such conditions.

Having thus disclosed our invention and described in detail representative examples of the best manner of practicing it, we claim and desire to secure by Letters Patent:

1. The method of treating wool to reduce its alkali solubility consisting essentially of the steps of contacting the wool with an aqueous solution of between about 0.3 and 10% by weight of acrolein and having a pH between about 2 and 7 for a time of less than 2 hours and at a temperature of less than 120° C., said time, temperature and concentration conditions being interrelated to produce a reduction in the alkali solubility of said wool, and drying said wool.

2. The method of treating wool to reduce its alkali solubility consisting essentially of the steps of contacting the wool with an aqueous solution of between about 0.3 and 10% by weight of acrolein and having a pH between

about 2 and 7 for a time of less than 2 hours and at a temperature of between about 65° C. and 100° C., said time, temperature and concentration conditions being interrelated to produce a reduction in the alkali solubility of said wool, and drying said wool.

3. The process defined by claim 1 wherein the wool is dried at a temperature between about 60° C. and 120° C.

4. The method of treating wool to reduce its alkali solubility consisting essentially of the steps of contacting the wool with an aqueous solution of about 3% by weight of acrolein and about 2% by weight of material selected from the group consisting of methacrolein and formaldehyde, for a time of less than 2 hours and a temperature of less than 120° C., said time, temperature and concentration conditions being interrelated to produce a reduction in the alkali solubility of said wool, and drying said wool.

#### References Cited in the file of this patent

| UNITED STATES PATENTS |           |               |
|-----------------------|-----------|---------------|
| 787,923               | Kann      | Apr. 25, 1905 |
| 2,322,486             | Swallen   | June 22, 1943 |
| 2,342,994             | Atwood    | Feb. 29, 1944 |
| 2,383,963             | Gottfried | Sept. 4, 1945 |
| 2,422,586             | Royer     | June 17, 1947 |
| 2,524,042             | Croston   | Oct. 3, 1950  |
| 2,583,574             | Jones     | Jan. 29, 1952 |
| 2,676,871             | McGovern  | Apr. 27, 1954 |

| FOREIGN PATENTS |         |               |
|-----------------|---------|---------------|
| 334,528         | Germany | Mar. 15, 1921 |
| 482,543         | Canada  | Apr. 15, 1952 |

#### OTHER REFERENCES

Parker et al.: J.S.D. and C., November 1947, Protecting Dyed Animal Fibers Against Harmful Effects of Discharging Agents, p. 362.